

E. W. WILKINSON.  
ORE CONCENTRATION.  
APPLICATION FILED DEC. 8, 1918.

1,398,990.

Patented Dec. 6, 1921.



Inventor  
Eltoft Wray Wilkinson  
By his Attorneys  
William & Hitchard

# UNITED STATES PATENT OFFICE.

ELTOFT WRAY WILKINSON, OF SAN FRANCISCO, CALIFORNIA, ASSIGNOR TO  
MINERALS SEPARATION NORTH AMERICAN CORPORATION, OF NEW YORK,  
N. Y., A CORPORATION OF MARYLAND.

## ORE CONCENTRATION.

1,398,990.

Specification of Letters Patent. Patented Dec. 6, 1921.

Application filed December 31, 1918. Serial No. 269,108.

To all whom it may concern:

Be it known that I, ELTOFT WRAY WILKINSON, a subject of the King of Great Britain, and resident of the city of San Francisco, county of San Francisco, and State of California, have invented certain new and useful Improvements in Ore Concentration, of which the following is a specification.

My invention relates to processes for concentrating ores or similar substances wherein, or upon the grinding of which, there are mixtures of solid substances having different physical properties, by utilizing these differences and the property possessed by certain agents of forming a froth with water or other liquid, the bubbles composing which have the ability of selecting the solid substances of one or more of the different classes and rejecting the remainder. These processes are widely utilized in the concentration of ores and other mineral substances, and the agents are commonly termed mineral-frothing agents. This term is therefore used herein to describe such agents. The processes are generally known as froth flotation processes.

The present invention relates more particularly to the mineral-frothing agents used in these processes and is applicable to all the different methods of bringing into action the useful properties of the mineral-frothing agent, the solid substances to be separated, and the gaseous bubbles.

I have found that by oxidizing mineral-frothing agents, such as the insoluble or oily mineral-frothing agents oleic acid or cotton-seed oil, by the agency of heat, a more efficient mineral-frothing agent is produced. The oxidation of the mineral-frothing agent is carried out by bringing it, either in the form of streams, globules, drops, spray, vapor or gas, together with oxygen or air, into a heated zone or region. Thereafter the products of the oxidation are subjected to condensation by methods already known. The condensation yields oily liquid, aqueous liquid and uncondensed gas or vapor. Each of the products is a mineral-frothing agent,—one may, however, be more effective as such than the others. Again the proportions of these products vary with different temperatures and with different propor-

tions of oxygen, and the temperature and the proportion of oxygen used depends on the nature of the material treated and the 55 nature and quantity of the particular product desired.

I shall now particularly describe examples of the carrying out of my invention with reference to the accompanying drawings, 60 which illustrate forms of apparatus that may be used in carrying out my invention, and shall thereafter point out my invention in claims.

Figure 1 is a diagrammatic view of an 65 apparatus for the treatment of frothing agents and the separation of the products thereof.

Fig. 2 is a diagram or flow sheet of the arrangement of complete apparatus for carrying out my invention.

I will first describe the apparatus shown in Fig. 1. Here *a* is a gas meter which measures the amount of air admitted to a retort *c* through a small tube *b*. This retort *c* is heated by a ring burner *q*. It comprises a copper cylinder permanently closed at the bottom and having a lid *f* bolted to a flange at the top. The small tube *b* from the gas meter *a* has a regulating valve *s* 80 therein and enters the retort through an opening in the lid *f* and terminates near the top of the retort. The material to be treated is supplied to the retort through a burette *d* from which a tube *e* extends down through the lid *f* and terminates near the bottom of the retort. A thermo-couple *g* is arranged in the retort near the bottom thereof and is connected by wires passing through the lid *f* to a voltmeter *h*, the thermo-couple 90 and voltmeter constituting a pyrometer for indicating the temperature maintained at the lower part of the retort. A tube *k* extends from the top of the retort through the lid and carries off the products. All of 95 these tubes and wires make tight joints with the lid. The tube *k* connects with a condenser *l* consisting of a coil tube *i* immersed in a water jacket. The condenser coil is connected at its other end by a tube *j* to 100 three condensing vessels *m<sup>1</sup>*, *m<sup>2</sup>*, *m<sup>3</sup>*, arranged in series, the tube *j* being the inlet tube of the first vessel and extending to near the bottom thereof. An outlet tube *j'* for the

first vessel  $m^1$  extends out near the top of the vessel  $m^1$  and enters and extends to near the bottom of the second vessel  $m^2$ , and an outlet tube  $j^2$  for the second vessel  $m^2$  extends from near the top thereof and enters and extends to near the bottom of the third vessel  $m^3$ , and an outlet tube  $j^3$  for the vessel  $m^3$  extends out near the top thereof and enters the final condensing vessel or scrubber  $n$ . The condensing vessels  $m^1$ ,  $m^2$ ,  $m^3$ , are immersed in a water bath in the vessel  $r$  for cooling them. The final condenser or scrubber  $n$  conveys the residual products in an upward direction through absorbent material such as absorbent cotton. From this scrubber a tube  $n^1$  passes to an air pump  $o$ , and from the outlet pipe  $p$  of the air pump the residual material in gaseous form is discharged from the treatment system and may be fed directly to the flotation machine, or stored for use, or allowed to escape to the atmosphere.

The following is an example of the carrying out of this invention with oleic acid of the kind known on the market as Baker's oleic acid. 250 cc. of this oleic acid are poured into the burette  $d$  and the retort is heated so that the pyrometer records a temperature of 1000° Fahr. The stop cock on the burette is then opened so that about 3 cc. of oil per minute flows into the retort, and thereupon the flow of air is started by the operation of the pump  $o$  at the rate of about 0.98 liters per minute. The temperature of the heated zone is maintained at about 1000° F. White fumes form and are condensed by the system above described, the condensed material being an oily condensed liquid and an aqueous condensed liquid. The air pump  $o$  exhausts an uncondensed remainder, which was found to be a good frothing agent.

A pulp was made of 500 grams of zinc ore from the Elm Orlu mine, Butte, Montana, ground to pass through a 65 mesh Tyler standard screen, and this was mixed with 1700 cc. of cold tap water. A pulp was made up in a slide machine and acidified with 18.1 pounds of sulfuric acid per ton (of 2000 lbs.) of ore. To this pulp was added 1.7 pounds of the oily condensed product obtained in the tubes  $m^1$ ,  $m^2$  and  $m^3$  per ton (of 2000 lbs.) of ore, and the whole was agitated at a speed of about 1600 R. P. M. for two minutes. An excellent froth rose to the top of the pulp, and after settling of the slimes, was removed. Water was added to make up the proper volume, and the pulp was again agitated for two minutes at the same speed. The slimes were settled as before, and the froth removed. Further water was added to make up the proper volume, and the pulp was given one minute more of agitation at the same speed, the slimes settled, and the froth removed.

65 These three froths were combined, weighed

and assayed as concentrates, and the residues were weighed and assayed as tailings, with the following metallurgical results:

| Products.         | Weight %. | Assay % zinc. | Percentage of total zinc. | 70 |
|-------------------|-----------|---------------|---------------------------|----|
| Heads.....        | 100.00    | 14.8          | 100.0                     |    |
| Concentrates..... | 39.43     | 35.0          | 93.4                      |    |
| Tailings.....     | 60.57     | 1.6           | 6.6                       |    |

75

In carrying out this invention in the apparatus above described with cottonseed oil which like oleic acid is a fatty acid-bearing substance, the cottonseed oil used was obtained from Eimer and Amend, New York. The retort was heated so that the pyrometer recorded a temperature of about 1000° Fahrenheit. The stop cock on the burette was then opened so that 4 cc. per minute, or 3.7 grams per minute of the cottonseed oil flowed into the retort. Thereupon a flow of air was started by the operation of the pump first at the rate of 9.6 liters per minute. The temperature as indicated by the pyrometer was maintained at about 1048° F. during the operation. White fumes formed in the apparatus and were condensed in the system described. A condensed oily liquid and a condensed aqueous liquid was obtained, and uncondensed gas or vapor was delivered at the pump outlet pipe  $p$ .

80

The oily condensed products so obtained were of a dark brown color and partially solid at 60° F., being fluid at about 130° F. The uncondensed products exhausted from the air pump  $o$  had a strong, unpleasant, acrid smell, and were very lacrymal. The proportions in which the different condensed products were obtained were as follows:

90

The first condensation obtained in the tubes  $m^1$ ,  $m^2$   $m^3$ , contained 56% by volume of the original cottonseed oil used, of which 28% was oily and 28% aqueous.

100

The second condensation obtained by compressing and blowing air through the absorbent cotton in the scrubber  $n$  measured 2.5% by volume of the cottonseed oil used in the operation.

110

There were thus produced 30.5% by volume of oily material and 28.0% of aqueous, making a total of 58.5%, by volume, of condensed products.

115

Both oily condensed products were found to give excellent results when used as frothing agents, as was the uncondensed gaseous exhaust from the air pump  $o$ . For example:

120

A pulp was made up of 700 grams of zinc ore from the Butte & Superior mine, Butte, Montana, crushed through 80 mesh Tyler standard screen, and cold tap water, acidified with sulfuric acid at the rate of 25 pounds per ton (of 2000 lbs.) of ore. There was added copper sulfate at the rate of 1 pound per ton of ore. This pulp was agitated in a laboratory flotation machine of

125

130

the subaeration type with 1.6 pounds per ton of the first condensed oily product produced by the above reaction.

Agitation was continued for twenty minutes and a good self-discharging froth was taken off continuously during this time, while air was admitted to the bottom of the flotation machine.

The concentrates were weighed and assayed, as were the tailings, with the following result:

| 15 | Products.         | Weight %. | Assays % zinc. |          | Percentage of total zinc. |
|----|-------------------|-----------|----------------|----------|---------------------------|
|    |                   |           | % Zn.          | % insol. |                           |
|    | Heads.....        | 100.0     | 9.74           |          | 100.0                     |
|    | Concentrates..... | 21.9      | 38.48          | 77.6     |                           |
|    | Tailings.....     | 78.1      | 2.67           | 22.4     |                           |

20 Another test was made with exactly the same flotation conditions as above, with the exception that in place of the condensed oily products the uncondensed gaseous exhaust from the air pump  $\sigma$  was fed into the pulp directly for two minutes, being followed by twenty minutes agitation with the admission of air alone at the bottom of the machine, with the following result:

| 30 | Products.         | Weight %. | Assays. |          | Percentage of total Zn. |
|----|-------------------|-----------|---------|----------|-------------------------|
|    |                   |           | % Zn.   | % insol. |                         |
|    | Heads.....        | 100.0     | 14.5    |          | 100.0                   |
|    | Concentrates..... | 34.5      | 43.4    | 21.7     | 100.0                   |
| 35 | Tailings.....     | 65.5      | Trace.  | .....    | Trace.                  |

40 Ordinary commercial operations with re-treatments of the concentrates would in each instance produce a higher grade of concentrate and an improved recovery.

Fig. 2 of the drawings illustrates an arrangement of complete apparatus for carrying out this invention in the form of a flow sheet with the parts correspondingly lettered, additionally showing a storage tank  $k^1$  and a flotation machine  $t$  receiving the stored oily liquid from the storage tank  $k^1$  and a flotation machine  $u$  receiving the gaseous material exhausted by the air pump  $\sigma$  through the outlet pipe  $p$ . The details of these apparatus have heretofore been sufficiently described, and obviously the nature and arrangement of the apparatus would be varied to suit the requirements of different installations and best carry out the process constituting this invention.

I claim:

1. The process of concentrating ores which consists in mixing with an ore pulp a mineral frothing agent obtained by subjecting a frothing agent to partial decomposition in the presence of oxygen with the production of substantial amounts of easily condensable material other than water and also bringing gaseous bubbles into contact with the

solid particles in the ore pulp so as to produce mineral-bearing froth, and separating the froth.

2. The process of concentrating ores which consists in mixing with an ore pulp a mineral frothing agent obtained by subjecting an insoluble frothing agent to partial decomposition in the presence of oxygen with the production of substantial amounts of easily condensable material other than water and also bringing gaseous bubbles into contact with the solid particles in the ore pulp so as to produce mineral-bearing froth, and separating the froth.

3. The process of concentrating ores which consists in mixing with an ore pulp a mineral frothing agent obtained by subjecting oleic acid to partial decomposition in the presence of oxygen with the production of substantial amounts of easily condensable material other than water and also bringing gaseous bubbles into contact with the solid particles in the ore pulp so as to produce mineral-bearing froth, and separating the froth.

4. The process of concentrating ores which consists in mixing with an ore pulp a mineral frothing agent obtained by subjecting a frothing agent to partial decomposition in the presence of oxygen with the production of substantial amounts of easily condensable material other than water and also bringing gaseous bubbles into contact with the solid particles in the ore pulp so as to produce mineral-bearing froth, and separating the froth.

5. The process of concentrating ores which consists in mixing with an ore pulp a mineral frothing agent obtained by subjecting an insoluble frothing agent to a partially decomposing heat in the presence of oxygen with the production of substantial amounts of easily condensable material other than water and also bringing gaseous bubbles into contact with the solid particles in the ore pulp so as to produce mineral-bearing froth, and separating the froth.

6. The process of concentrating ores which consists in mixing with an ore pulp a product obtained by subjecting oleic acid to a partially decomposing heat in the presence of oxygen and also bringing gaseous bubbles into contact with the solid particles in the ore pulp so as to produce mineral-bearing froth, and separating the froth.

7. The process of concentrating ores which consists in mixing with an ore pulp a mineral frothing agent obtained by subjecting a fatty acid-bearing substance to a partially decomposing heat in the presence of oxygen to effect substantial oxidation thereof and also bringing gaseous bubbles into contact with the solid particles in the ore pulp so as to produce mineral-bearing froth, and separating the froth.

8. The process of concentrating ores which consists in mixing with an ore pulp a mineral frothing agent obtained by subjecting an insolubly fatty acid-bearing substance to a partially decomposing heat in the presence of oxygen to effect substantial oxidation thereof and also bringing gaseous bubbles into contact with the solid particles in the ore pulp so as to produce mineral-bearing froth, and separating the froth.
9. The process of concentrating ores which consists in mixing with an ore pulp an oily product obtained by subjecting oleic acid to substantial oxidation by heat in the presence of oxygen to effect substantial oxidation thereof and also bringing gaseous bubbles into contact with the solid particles in the ore pulp so as to produce mineral-bearing froth, and separating the froth.
10. The process of concentrating ores which consists in mixing with an ore pulp an oily distillate obtained by subjecting a fatty acid-bearing substance to a partially decomposing heat in the presence of oxygen to effect substantial oxidation thereof and

also bringing gaseous bubbles into contact with the solid particles in the ore pulp so as to produce mineral-bearing froth, and separating the froth.

11. The process of concentrating ores 30 which consists in mixing with an ore pulp an oily distillate obtained by subjecting a fatty acid-bearing substance to a partially decomposing heat in the presence of oxygen to effect substantial oxidation thereof and 35 also bringing gaseous bubbles into contact with the solid particles in the ore pulp so as to produce mineral-bearing froth, and separating the froth.

12. The process of concentrating ores 40 which consists in mixing with an ore pulp an oily distillate obtained by subjecting oleic acid to partial decomposition in the presence of oxygen and also bringing gaseous bubbles into contact with the solid particles in the ore pulp so as to produce mineral-bearing froth, and separating the froth.

In testimony whereof, I have affixed my signature to this specification.

ELTOFT WRAY WILKINSON.